# EUROPEAN PATENT SPECIFICATION

(11) **EP 3 377 659 B1**
(45) Date of publication and mention of the grant of the patent: **16.12.2020**
(21) Application number: 16847594.5
(22) Date of filing: 18.11.2016
(51) Int. Cl.: C22B 1/245, C22B 34/12

(54) **IMPROVED ILMENITE SMELTING PROCESS**
VERBESSERTES ILMENITSCHMELZVERFAHREN
PROCÉDÉ DE FUSION D'ILMÉNITE AMÉLIORÉ

(30) Priority: 18.11.2015 ZA 201508501
(43) Date of publication of application: 26.09.2018
(73) Proprietor: Mintek, 2194 Randburg (ZA)
(72) Inventor: BISAKA, Kabwika, 2194 Randburg (ZA); GOSO, Xolisa, 2194 Randburg (ZA); THOBADI, Itumeleng, 2194 Randburg (ZA)
(74) Representative: Tomkinson, Alexandra
(86) International application number: PCT/ZA2016/050049
(87) International publication number: WO 2017/087997

(56) References cited:
- CN-A- 103 451 454
- US-A- 3 765 868
- US-B1- 6 685 761
- XU M ET AL: "Beneficiation of Titanium Oxides From Ilmenite by Self-Reduction of Coal Bearing Pellets", JOURNAL OF IRON AND STEEL RESEARCH INTERNATIONAL, GANGTIE YANJIU XUEBAO, CN, vol. 13, no. 2, 1 March 2006 (2006-03-01), pages 6-9, XP022933365, ISSN: 1006-706X, DOI: 10.1016/S1006-706X(06)60033-2 [retrieved on 2006-03-01]

## Description

### BACKGROUND OF THE INVENTION

This invention relates to a consolidated process for the preparation of carbon-based ilmenite pellets, the solid-state reduction thereof, and the subsequent smelting thereof in an electric furnace.

The smelting of ilmenite consumes substantial quantities of electrical energy. Additionally, the operability of the furnace can be hindered due to frothing effects.

Feed to the smelting furnace is generally made up of raw ilmenite ore and a solid, carbonaceous reductant. Raw ilmenite, in a particular process, is replaced by pre-reduced ilmenite pellets. The steps for the production process of the latter are to prepare ilmenite pellets using bentonite and to pre-reduce the pellets in a rotary kiln in the presence of a solid, carbonaceous reductant in excess. The smelting of the pre-reduced ilmenite pellets is thus carried out in an AC furnace. The TiO₂ slag produced in this way is, however, contaminated with the bentonite which is an inorganic binder.

US 6 685 761 relates to a method of and apparatus for producing beneficiated titanium oxides. The method includes the steps of forming agglomerates using a binder such as cellulose or fibre of carbon-based materials and low grade titanium materials, containing iron and iron oxides, and pre-reducing the agglomerates with heat to produce pre-reduced agglomerates of titanium oxides and metallized carbon-containing iron. Subsequently the pre-reduced agglomerates are heated in a hearth furnace to complete the reduction of oxides of titanium and to complete the metallization of the carbon-containing iron. The molten agglomerate is discharged into an electric smelter to provide a molten iron product and beneficiated titanium oxide slag. The high carbon molten iron product is then purified. The method also provides for the inclusion of a binder in the agglomerate, e.g. cellulose fiber.

An object of the present invention is to provide an alternative process for pre-reducing an ore essentially targeting the metallisation of iron oxides contained in the ore.

### SUMMARY OF THE INVENTION

The invention provides a method of preparing a pre-reduced ilmenite ore for smelting, wherein metal oxides contained in the ore are selectively reduced in solid-state reactions over titanium oxide, the method being characterised in that it includes the step of pre-reducing carbon-based pellets of the ore wherein the pellets are less than 6mm in size and are prepared from a blend of the ore, coal fines and an organic binder.

The metal oxides, other than titanium oxides, in the pellets may be pre-reduced to a maximum extent i.e. essentially fully or they may be partially pre-reduced.

The pellets may be in a range of 2mm to 5mm.

The coal fines used to prepare the pellets may be of -106 microns.

The ratio of the coal to the metallic oxide content may be practically determined. For example a stoichiometric ratio for the full reduction of iron in the ore can be used.

The organic binder content may lie in the range of 0 to 1%. This content may be dictated by the physical properties of the resulting pellets principally the strength of the pellets in a green state and in an air-dried or indurated state. The pellets may be may be air-indurated for at least 4 days. This period is usually adequate to ensure that the pellets are sufficiently strong to allow their safe and efficient handling to subsequent pre-reduction reactors. The mechanical strength of the pellets is preferably above 600N. The pellets should also have an acceptable behaviour in a hot reactor environment to avoid decrepitation due to excessive swelling.

A single binder or a mixture of binders may be used. The invention is not limited in this respect.

Pre-reduced pellets are evaluated based on the reduction extent of iron oxides contained in the ore. Preferably the iron oxide should be present in a quantity of less than 10% from the initial content. However a consistent pre-reduction yield should be a main target during a normal and stable operation.

The pellets may be subjected to a thermal reduction process or to a hybrid, solid-state, reduction process.

The pellets, air-dried and indurated, may be heated in a fixed bed reactor at an optimal residence time which may lie in a range of from 0.5 to 4 hours.

If a thermal pre-reduction step is adopted then the pellets may be heated at a temperature in the range of 1100 to 1200°C.

If the hybrid, solid-state, pre-reduction step is adopted then the pellets may be heated to a temperature in the range of 900 to 1000°C in a controlled atmosphere of a reducing gas.

The reducing gas may comprise one or more of the following: CO, syngas (CO + H₂), natural gas and hydrogen.

If a fixed bed reactor is employed then the reducing gas may be filtered through a hot burden in the reactor. The reducing gas flowrate should be selected to achieve an adequate reduction yield of the iron oxides in the ore, as well as acceptable reactor operation performance.

The invention finds particular application in the preparation of pre-reduced, carbon-based, ilmenite micro-pellets which are to be smelted e.g. in a DC open arc furnace. However, the principles of the invention may be employed for the pre-reduction of pellets of titaniferous magnetite, ferrochrome and ferromanganese ores for the subsequent production of titania slag, chrome and manganese, alloys respectively.

Reference has been made to heating the air-dried pellets in a fixed bed reactor. This is exemplary only and non-limiting. A moving bed and a rotary kiln may be employed in place of the fixed bed reactor, in a pre-reduction stage. It is important that abrasion of the pellets is minimised and it should be possible to separate pre-reduced fines from other material, for example through the use of magnetic or equivalent techniques.

### BRIEF DESCRIPTION OF THE DRAWING

The invention is further described by way of example with reference to the accompanying figures wherein;
Figure 1 illustrates in flow chart form the pre-reduction of carbon-based, ilmenite micro-pellets and the subsequent smelting thereof;
Figure 2 is a diagram depicting an impact of the residence time on pre-reduction and metallisation degrees at 1000°C and 0.5l CO / min; and
Figure 3 is a diagram depicting an impact of the CO flowrate on the pre-reduction and metallisation degrees at 1000°C and 1h residence time.

### DESCRIPTION OF PREFERRED EMBODIMENT

The invention is hereinafter described with reference to the pre-reduction of carbon-based, ilmenite, micro-pellets. Although this is a preferred application of the principles of the invention it is possible to adapt the principles described herein for the pre-reduction of titaniferous magnetite, ferrochrome and ferromanganese ores.

Raw ilmenite ore 10 of a suitable size is fed to a blender 12. The blender also receives coal fines 14 of -106 micron in size and an organic binder 16 formed from a single binder or from a mixed binder composition.

The ratio of the input coal to the ilmenite is determined taking into account practical considerations. For instance a stoichiometric ratio which achieves a full reduction of iron in the ilmenite ore can be used. Further, the input of organic binder or mixes of organic binders, in the range of up to 1%, is dictated by the physical properties of the resulting pellets, particularly the green and air-dried strengths of the pellets. The resulting pellets should also have an acceptable behaviour (subsequently) in a hot reactor environment to avoid decrepitation due to excessive swelling.

The blender 12 produces carbon-based, ilmenite, micro-pellets of 2mm to 5mm in size. These pellets are then air-dried (step 20).

The air-dried, indurated pellets are then subjected to a thermal pre-reduction step 22, or to a hybrid, solid-state pre-reduction step 24. In each instance the air-dried indurated pellets are heated in a fixed bed reactor 26 for an optimal residence time, generally from 0.5 to 4 hours.

If use is made of the thermal pre-reduction process the pellets are heated in the reactor 26 to a temperature in the range of 1100 to 1200°C. If use is made of the hybrid approach then the pellets are heated in the reactor 26 to a temperature of 900 to 1000°C in a controlled atmosphere of a reducing gas 30 which comprises one or more of CO, syngas, natural gas and hydrogen. The reducing gas is filtered through the hot burden of the pellets in the reactor 26. The reducing gas flowrate is regulated to achieve an adequate pre-reduction yield. The flowrate should also be regulated to optimise the reactor operation, principally the thermal efficiency and the production cost.

Process parameters of importance, in respect of the of pre-reduction technique used, include: the ilmenite grain size distribution, the composition of the pellets, the sizes of the pellets, the operating temperature, the residence time and the reducing gas flowrate.

Taken under consistent operating conditions each method is able to produce a consistent pre-reduction yield. The hybrid method, despite operating at a lower temperature then the thermal reduction method, appears to offer a higher pre-reduction yield than the thermal method.

The fully or partially pre-reduced ilmenite pellets 32, emerging from the reactor 26, can be fed, cold or hot, to a conventional ilmenite smelting process 36.

Without being bound by the following explanation it is believed that the organic binder provides a more intimate contact between the ilmenite and the coal fines. The small pellet size feature, in a highly reducing atmosphere, assists the transfer of heat and mass in the diffusion of gaseous reductants, such as CO and H₂, to the reaction sites. The organic binder 16 burns off at the process temperature, a feature which induces localised reduction and promotes the formation of cracks and pores in the ilmenite ore grains contained in the pellets 32. The specific surface areas of the ilmenite pellets are therefore increased and the diffusion rate of the gas reductant to the reaction sites is enhanced. This in turn impacts on the pre-reduction yield. The reduction process can be smoothly and efficiently operated despite the minor sintering of the pellets that may occur at elevated temperatures.

The fully or partially pre-reduced, carbon-based ilmenite pellets which are fed, either hot or cold, into a DC open arc furnace decrease the consumption of electricity in the furnace, help to address slag foaming and result in an improved grade of TiO₂ slag 38 output by the furnace.

Through tests it has been established that iron oxide in the pellets was nearly completely reduced through the use of the hybrid pre-reduction process carried out at a temperature of 1000°C and for a residence time of 2 hours. The pre-reduction yield was increased as temperature, residence time and reducing gas flowrate were increased.

The use of the thermal pre-reduction process at a temperature of 1100 to 1200°C produced a pre-reduction yield of about 85% - a value which is adversely affected with an increase in ilmenite ore grain size and with an increase in the size of the coal fines.

About 4 tons of cold pre-reduced ilmenite pellets were smelted in a DC open arc furnace. The energy consumption of the furnace lay in the range of 0.6 to 0.7 kWh / kg of pre-reduced ilmenite pellets - a figure which represents an electrical energy saving of 30 to 40% compared to a conventional ilmenite smelting process. The smelting process was stable with no visible sign of foaming. The product contained about 95% TiO₂ and about 3% FeO.

A higher grade TiO₂ slag (above 90%) can thus be achieved, using conventional ilmenite feedstock in smelting operations, with no foaming occurring. Using the method of the current invention, a lower grade ilmenite could be used as feedstock to produce TiO₂ slag of at least 85% TiO₂ content.

The invention has been described with reference to the use of a gaseous reductant. It is possible though to make use of a solid reductant such as anthracite or coal, instead of the reducing gas 30. Also the reactor 26 which, typically, is a fixed bed reactor can be replaced by a moving bed or by a rotary kiln configuration provided abrasion effects between the pellets are minimised. It should be possible though to separate the pre-reduced pellets, for example using magnetic techniques, from the other material emerging from the reactor.

Additional carbonaceous solid reductant can be used in excess to reduce residual iron in the slag to below 6% without inducing slag foaming.

### DESCRIPTION OF A PILOT TEST OF THE PROCESS OF THE INVENTION

A 200 kW DC arc furnace facility was used for demonstrating the smelting of pre-reduced ilmenite pellets. The furnace had a 1 m outer diameter, water-spray cooled steel shell lined with a single layer and three rows of magnesite-chrome bricks and a hearth lined with rammable magnesia. The refractory lining resulted in the furnace crucible internal diameter (ID) of 0.656 m. The furnace was equipped with an alumina lined conical roof and a shell bolted on a domed base. A single taphole was used to tap a stream of both molten slag and metal. The furnace was equipped with a single and centrally-located graphite electrode of 40 mm diameter operating as a cathode while the anode comprised steel pins buried in the hearth. The feed system comprised individual hoppers used to feed anthracite and pre-reduced ilmenite pellets through a furnace feed pipe. The furnace was equipped with an off-gas system for the cleaning of produced process gas prior to release thereof into the atmosphere.

Carbon-based ilmenite pellets containing the as received ilmenite, stoichiometric amount of anthracite, were prepared using a proprietary organic binder at a required dosage. The as-received ilmenite had a particle size distribution of D₁₀₀ in the 38 µm to 150 µm size range. The anthracite was milled to a D₈₅ passing 106 µm to facilitate its incorporation into an ilmenite pellet recipe. Pellets were prepared in a pilot-scale pelletizing unit comprising an inclined rotating pan of 985 mm diameter and 170 mm depth. The mechanical strengths of the pellets were measured and found to vary with the type and dosage of binder used, within a range of 0.01 - 0.03 MPa for green pellets and 0.81 - 1.50 MPa for indurated pellets at ambient conditions.

Batches of 250 kg each of indurated pellets were reduced in an electrically heated muffle furnace operated at a controlled temperature of 1100 °C. During a three hour firing time, in total 5 kg of CO was blown intermittently through the reactor burden at intervals of 10 minutes. The pellets were loaded in a single tray of 1700 mm x 900 mm, having a loading area of a mesh screen acting as a distribution plenum for the reducing gas.

Both the raw and pre-reduced ilmenite materials at various conditions were chemically analysed; specifically an analysis of the iron oxidation states (Fe³⁺, Fe²⁺, and Fe⁰) was used to calculate the pre-reduction and metallisation yields for the pellets. Negligible reduction of titanium oxides was assumed throughout and the pre-reduction yield was therefore calculated based on the mass balance of oxygen associated with each gram of iron before and after pre-reduction. Equations [1] and [2] were used for the calculation of the prereduction and metallization yields, respectively. $Pr e - reduction yield = 100 \times \frac{\left(Oxygen removed by the pre-reduction process\right)}{\left(Oxygen associated with each gram of iron in the ilmenite sample\right)}$ $Metallisation yield = 100 \times \frac{{Fe}^{0}}{{Fe}_{metal}}$

The chemical analyses of the ore and anthracite are summarised in Table 1 and Table 2, respectively.

**Table 1: Bulk chemical composition of the raw ilmenite (mass %)**

| **MgO** | **Al₂O₃** | **SiO₂** | **CaO** | **TiO₂** | **V₂O₅** | **Cr₂O₃** | **MnO** | **FeO** | **Fe²⁺** | **Fe⁰** | **Fe/Ti** |
|---|---|---|---|---|---|---|---|---|---|---|---|
| 0.28 | 0.44 | 0.57 | 0.05 | 46.6 | 0.25 | 0.09 | 1.08 | 47.87 | 13.50 | <0.05 | 1.33 |

| | | | | | | | | | | | |
|---|---|---|---|---|---|---|---|---|---|---|---|
| <0.05%: the analyte concentration could not be accurately quantified as it is below the limit of detection (LOD) Total Fe in the sample is expressed as % FeO | | | | | | | | | | | |

**Table 2: Summary of the bulk chemical composition of the anthracite (mass %)**

| **Moisture** | **Ash** | **Volatile** | **Fixed carbon** | **Total carbon** | **Total sulphur** |
|---|---|---|---|---|---|
| 3.57 | 4.74 | 6.19 | 89.1 | 90.7 | 0.56 |

In total, about 3.6 tons of pre-reduced pellets were produced. The pellets were bagged in 1 m³ bags from which five composite samples were collected. The chemical analyses of the 5 composite samples are given in Table 3.

**Table 3: Chemical compositions of the pre-reduced pellets**

| | MgO | Al₂O₃ | SiO₂ | CaO | TiO₂ | V₂O₅ | Cr₂O₃ | MnO | Total Fe | Fe⁰ | Fe²⁺ | C | Ti³⁺ | Fe/Ti ratio |
|---|---|---|---|---|---|---|---|---|---|---|---|---|---|---|
| TP Bag 1 | 0.53 | 0.33 | 0.31 | 0.10 | 44.4 | 0.36 | 0.07 | 1.05 | 34.92 | 25.55 | 9.37 | 7.23 | 6.55 | 1.32 |
| TP Bag 2 | 0.55 | 0.30 | 0.26 | 0.07 | 44.5 | 0.36 | 0.08 | 1.06 | 35.23 | 25.44 | 9.79 | 7.72 | 6.76 | 1.32 |
| TP Bag 3 | 0.50 | 0.30 | 0.24 | 0.15 | 43.5 | 0.33 | 0.07 | 1.03 | 33.60 | 21.90 | 11.7 | 7.97 | 5.45 | 1.29 |
| TP Bag 4 | 0.48 | 0.32 | 0.39 | 0.11 | 42.4 | 0.33 | 0.07 | 1.05 | 34.46 | 22.66 | 11.8 | 8.01 | 4.78 | 1.35 |
| TP Bag 5 | 0.36 | 0.45 | 0.64 | 0.18 | 41.9 | 0.33 | 0.07 | 1.08 | 36.01 | 24.21 | 11.8 | 7.20 | 4.66 | 1.43 |
| Average | 0.48 | 0.34 | 0.37 | 0.12 | 43.3 | 0.34 | 0.07 | 1.05 | 34.84 | 23.95 | 10.8 9 | 7.63 | 5.64 | 1.32 |
| St dev | 0.07 | 0.06 | 0.16 | 0.04 | 1.17 | 0.02 | 0.004 | 0.02 | 0.90 | 1.64 | 1.21 | 0.39 | 0.98 | 0.02 |

The calculated degrees of prereduction and metallization for the five composite samples are presented in Table 4

**Table 4: Pre-reduction and metallisation degrees of ilmenite pellets**

| Composite sample no. | Pre-reduction degree, % | Metallisation degree, % |
|---|---|---|
| 1 | 79.7 | 73.2 |
| 2 | 78.9 | 72.2 |
| 3 | 73.6 | 65.2 |
| 4 | 74.1 | 65.8 |
| 5 | 75.1 | 67.2 |
| Average | 76.3 | 68.7 |
| St dev | 2.8 | 3.7 |

Tables 3 and 4 show that pellets prereduced to a consistent extent were produced as a result of the uniform furnace operating conditions.

Results from laboratory tests in a tube reactor of 80 mm diameter showed a very important feature of this process that is presented in Figures 2 and 3. Tests conducted at a temperature of 1000°C, showed that pre-reduction and metallisation degrees are both related to the residence time and CO flowrate. Increasing the CO flowrate appears to positively affect the yields, suggesting that CO diffusion would play a significant role in this process.

Continuous smelting of partially reduced ilmenite pellets (approx.. 70% prereduction yield) was carried out to demonstrate stable furnace operation as well as production of a consistent slag quality, in particular, a slag TiO₂ grade above 85%. The test work also had the objective of confirming the process specific energy requirement. The slag results are presented in Table 5.

**Table 5: Analysis of slag from the stable smelting operation, in mass %**

| **Tap** | ***TiO₂** | **CT₂O₃** | **MnO** | **FeO** | **V₂O₅** | **SiO₂** | **CaO** | **Al₂O₃** | **MgO** |
|---|---|---|---|---|---|---|---|---|---|
| A | 84.74 | 1,34 | 1,37 | 2,06 | 0,30 | 1,31 | 0,34 | 1,96 | 6,58 |
| B | 87.84 | 0,60 | 1,18 | 2,59 | 0,21 | 1,16 | 0,28 | 2,49 | 3,65 |
| C | 83.15 | 0,31 | 1,68 | 2,73 | 0,29 | 1,20 | 0,38 | 2,76 | 7,50 |
| D | 88.86 | 0,45 | 0,68 | 4,89 | 0,17 | 0,49 | 0,31 | 1,45 | 2,70 |
| E | 88.19 | 0,45 | 0,99 | 4,37 | 0,16 | 0,43 | 0,35 | 1,53 | 3,53 |
| F | 91.27 | 0,31 | 1,47 | 1,58 | 0,15 | 0,28 | 0,32 | 1,47 | 3,15 |
| G | 94.28 | 0,08 | 1,32 | 1,25 | 0,10 | 0,21 | 0,17 | 0,98 | 1,61 |
| H | 93.32 | 0,09 | 1,21 | 1,48 | 0,10 | 0,16 | 0,14 | 1,10 | 2,40 |

| | | | | | | | | | |
|---|---|---|---|---|---|---|---|---|---|
| *by difference | | | | | | | | | |

**Table 6: Evolution of composition of pig iron from the stable smelting operation, in mass %**

| **Tap** | **Fe** | **Ti** | **V** | **Si** | **Cr** | **Mn** | **C** | **P** | **S** |
|---|---|---|---|---|---|---|---|---|---|
| A | 95.54 | 0.67 | 0.24 | 0.34 | 1.04 | 0.48 | 1.66 | 0.02 | 0.01 |
| B | 95.92 | 0.43 | 0.23 | 0.36 | 1.08 | 0.44 | 1.53 | 0.00 | 0.01 |
| C | 95.15 | 0.55 | 0.16 | 0.38 | 1.47 | 0.33 | 1.92 | 0.02 | 0.02 |
| D | 97.03 | 0.16 | 0.09 | 0.18 | 0.52 | 0.21 | 1.76 | 0.02 | 0.03 |
| E | 94.59 | 0.29 | 0.20 | 0.62 | 1.14 | 0.51 | 2.57 | 0.03 | 0.05 |
| F | 91.81 | 3.64 | 0.23 | 0.64 | 1.17 | 0.86 | 1.62 | 0.01 | 0.02 |
| G | 95.83 | 0.57 | 0.20 | 0.41 | 0.71 | 0.60 | 1.64 | 0.02 | 0.02 |
| H | 93.66 | 1.34 | 0.32 | 1.28 | 0.89 | 0.88 | 1.56 | 0.02 | 0.05 |

Slag FeO contents as low as 1.3 % were achieved without visible signs of slag foaming. This condition was maintained for a longer period during which stable furnace operation was demonstrated and slags of consistent FeO content were produced. Results for this particular test work suggest that smelting of partially reduced ilmenite and operating the furnace with lower FeO content in the slag are technically possible.

The 200 kW DC open-arc furnace was operated at a power level in the range of 115 - 140 kW and at a corresponding voltage of 100 - 115 V. Consistent furnace heat losses in the range of 60 - 90 kW were measured. Average tapping temperatures measured using an optical pyrometer were scattered within a range between 1670 and 1780°C. The specific energy requirement (SER) for the smelting of prereduced carbon-based pellets was measured between 0.6 and 0.7 kWh / kg prereduced ilmenite. A 30-40 % reduction in furnace electricity required relative to a conventional smelting process can be achieved assuming that a prereduction yield of at least 70 % can be achieved. Arc resistivities were measured for various conditions investigated in order to predict the furnace arc stability. Arc resistivity was found to be in the range of 0.0168 and 0.0240 Ω.cm which range is close to 0.0175 Ω.cm, a typical value for arc resistivity in smelting processes with CO-rich atmospheres (in the absence of foaming).

## Claims

1. A method of preparing a pre-reduced ilmenite ore (32) for smelting (36) wherein metal oxides, contained in the ore are selectively reduced in solid-state reactions over titanium oxide, the method includes the step of pre-reducing (22 and 24) carbon-based pellets (21) of the ore, wherein the pellets are less than 6mm in size and are prepared from a blend of the ore (10), coal fines (14) and an organic binder (16).

2. A method according to claim 1 **characterised in that** the metal oxides, other than titanium oxides, in the pellets are pre-reduced to a maximum extent.

3. A method according to claim 1 **characterised in that** the pellets are between 2mm and 5mm in size.

4. A method according to claim 1 **characterised in that** the coal fines (14) have a size of -106 microns.

5. A method according to any one of claims 1 to 4 **characterised in that** the ratio of the coal to the metallic oxide content is determined using a stoichiometric ratio for the full reduction of iron in the ore.

6. A method according to any one of claims 1 to 5 **characterised in that** the organic binder (16) content is in the range of 0 to 1%.

7. A method according to any one of claims 1 to 6 **characterised in that** a single organic binder (16) or a mixture of organic binders (16) is used.

8. A method according to any one of claims 1 to 7 **characterised in that** the pellets are air indurated (20) for at least 4 days.

9. A method according to claim 8 **characterised in that** a mechanical strength of the pellets (21) is of the order of 600N.

10. A method according to any one of claims 1 to 9 **characterised in that** iron oxide in the ore (10) is present in a quantity of less than 10%.

11. A method according to any one of claims 1 to 10 **characterised in that** the pellets are subjected to a thermal reduction process (22) or to a hybrid, solid-state, reduction process (24).

12. A method according to claim 11 **characterised in that** the pellets are heated in a fixed bed reactor (26) for a time period of between 0.5 to 4 hours.

13. A method according to claim 12 **characterised in that** a thermal pre-reduction step (22) is adopted and the pellets (21) are heated to a temperature in the range of 1100 to 1200°C.

14. A method according to claim 11 or 12 **characterised in that** a hybrid, solid-state, pre-reduction step 24 is adopted and the pellets (21) are heated to a temperature in the range of 900 to1000°C.

15. A method according to claim 14 **characterised in that** a reducing gas (30) is filtered through a hot burden in the fixed bed reactor (26).

16. A method according to claim 15 **characterised in that** the reducing gas (30) comprises one or more of the following: carbon monoxide; syngas (CO+H2); natural gas; and hydrogen.

17. A method according to any one of claims 1 to 16 **characterised in that** the smelting is conducted in a DC open arc furnace at a temperature of between 1650 and 1750°C.

## Patentansprüche

1. Verfahren zur Herstellung eines vorreduzierten Ilmeniterzes (32) zur Verhüttung (36), wobei in dem Erz enthaltene Metalloxide in Festkörperreaktionen über Titanoxid selektiv reduziert werden, wobei das Verfahren den Schritt des Vorreduzierens (22 und 24) von Pellets (21) des Erzes auf Kohlenstoffbasis beinhaltet, wobei die Pellets eine Größe von weniger als 6 mm haben und aus einem Gemisch des Erzes (10), Staubkohle (14) und einem organischen Bindemittel (16) hergestellt werden.

2. Verfahren nach Anspruch 1, **dadurch gekennzeichnet, dass** die Metalloxide außer Titanoxiden in maximalem Maße vorreduziert werden.

3. Verfahren nach Anspruch 1, **dadurch gekennzeichnet, dass** die Pellets eine Größe zwischen 2 mm und 5 mm haben.

4. Verfahren nach Anspruch 1, **dadurch gekennzeichnet, dass** die Staubkohleteilchen (14) eine Größe von -106 Mikrometer haben.

5. Verfahren nach einem der Ansprüche 1 bis 4, **dadurch gekennzeichnet, dass** das Verhältnis der Kohle zum Anteil von Metalloxid unter Verwendung eines stöchiometrischen Verhältnisses für die volle Reduktion von Eisen in dem Erz bestimmt wird.

6. Verfahren nach einem der Ansprüche 1 bis 5, **dadurch gekennzeichnet, dass** der Anteil des organischen Bindemittels (16) im Bereich von 0 bis 1 % ist.

7. Verfahren nach einem der Ansprüche 1 bis 6, **dadurch gekennzeichnet, dass** ein einzelnes organisches Bindemittel (16) oder eine Mischung organischer Bindemittel (16) verwendet wird.

8. Verfahren nach einem der Ansprüche 1 bis 7, **dadurch gekennzeichnet, dass** die Pellets wenigstens 4 Tage lang luftgehärtet (20) werden.

9. Verfahren nach Anspruch 8, **dadurch gekennzeichnet, dass** eine mechanische Festigkeit der Pellets (21) in der Größenordnung von 600 N ist.

10. Verfahren nach einem der Ansprüche 1 bis 9, **dadurch gekennzeichnet, dass** Eisenoxid in dem Erz (10) in einer Menge von weniger als 10 % vorhanden ist.

11. Verfahren nach einem der Ansprüche 1 bis 10, **dadurch gekennzeichnet, dass** die Pellets einem thermischen Reduktionsprozess (22) oder einem Hybrid-Festkörper-Reduktionsprozess (24) unterzogen werden.

12. Verfahren nach Anspruch 11, **dadurch gekennzeichnet, dass** die Pellets in einem Festbettreaktor (26) für eine Zeitspanne zwischen 0,5 und 4 Stunden erhitzt werden.

13. Verfahren nach Anspruch 12, **dadurch gekennzeichnet, dass** ein thermischer Vorreduktionsschritt (22) angewendet wird und die Pellets (21) auf eine Temperatur im Bereich von 1100 bis 1200 °C erhitzt werden.

14. Verfahren nach Anspruch 11 oder 12, **dadurch gekennzeichnet, dass** ein Hybrid-Festkörper-Vorreduzierungsschritt (24) angewendet wird und die Pellets (21) auf eine Temperatur im Bereich von 900 bis 1000 °C erhitzt werden.

15. Verfahren nach Anspruch 14, **dadurch gekennzeichnet, dass** ein reduzierendes Gas (30) durch einen heißen Möller im Festbettreaktor (26) gefiltert wird.

16. Verfahren nach Anspruch 15, **dadurch gekennzeichnet, dass** das reduzierende Gas (30) ein oder mehr der Folgenden aufweist: Kohlenmonoxid; Synthesegas (CO+H2); Erdgas; und Wasserstoff.

17. Verfahren nach einem der Ansprüche 1 bis 16, **dadurch gekennzeichnet, dass** die Verhüttung in einem offenen Gleichstrom-Lichtbogenofen bei einer Temperatur zwischen 1650 und 1750 °C erfolgt.

## Revendications

1. Procédé de préparation d'un minerai d'ilménite pré-réduit (32) en vue d'une fusion (36) dans lequel des oxydes de métal, contenus dans le minerai, sont réduits sélectivement dans des réactions à l'état solide sur de l'oxyde de titane, le procédé incluant l'étape de pré-réduction (22 et 24) de boulettes à base de carbone (21) du minerai, les boulettes ayant une taille inférieure à 6 mm et étant préparées à partir d'un mélange composé du minerai (10), de fines de charbon (14) et d'un liant organique (16).

2. Procédé selon la revendication 1 **caractérisé en ce que** les oxydes de métal, autres que des oxydes de titane, dans les boulettes sont pré-réduits jusqu'à une mesure maximale.

3. Procédé selon la revendication 1 **caractérisé en ce que** les boulettes ont une taille située entre 2 mm et 5 mm.

4. Procédé selon la revendication 1 **caractérisé en ce que** les fines de charbon (14) ont une taille de -106 microns.

5. Procédé selon l'une quelconque des revendications 1 à 4 **caractérisé en ce que** le rapport du charbon à la teneur en oxyde métallique est déterminé grâce à l'utilisation d'un rapport stœchiométrique pour la réduction complète du fer dans le minerai.

6. Procédé selon l'une quelconque des revendications 1 à 5 **caractérisé en ce que** la teneur en liant organique (16) se situe dans la gamme de 0 à 1 %.

7. Procédé selon l'une quelconque des revendications 1 à 6 **caractérisé en ce qu'**un seul liant organique (16) ou un mélange de liants organiques (16) est utilisé.

8. Procédé selon l'une quelconque des revendications 1 à 7 **caractérisé en ce que** les boulettes sont indurées à l'air (20) pendant au moins 4 jours.

9. Procédé selon la revendication 8 **caractérisé en ce qu'**une résistance mécanique des boulettes (21) est de l'ordre de 600 N.

10. Procédé selon l'une quelconque des revendications 1 à 9 **caractérisé en ce que** l'oxyde de fer dans le minerai (10) est présent dans une quantité inférieure à 10 %.

11. Procédé selon l'une quelconque des revendications 1 à 10 **caractérisé en ce que** les boulettes sont soumises à un processus de réduction thermique (22) ou à un processus de réduction hybride à l'état solide (24).

12. Procédé selon la revendication 11 **caractérisé en ce que** les boulettes sont chauffées dans un réacteur à lit fixe (26) pendant un intervalle de temps entre 0,5 à 4 heures.

13. Procédé selon la revendication 12 **caractérisé en ce que** l'étape de pré-réduction thermique (22) est adoptée et les boulettes (21) sont chauffées jusqu'à une température dans la gamme de 1100 à 1200 °C.

14. Procédé selon la revendication 11 ou 12 **caractérisé en ce qu'**une étape de pré-réduction hybride à l'état solide (24) est adoptée et que les boulettes (21) sont chauffées jusqu'à une température dans la gamme de 900 à 1000 °C.

15. Procédé selon la revendication 14 **caractérisé en ce qu'**un gaz de réduction (30) est filtré à travers un lit de fusion chaud dans le réacteur à lit fixe (26).

16. Procédé selon la revendication 15 **caractérisé en ce que** le gaz de réduction (30) comprend une ou plusieurs des substances suivantes : monoxyde de carbone ; gaz synthétique (CO + H2) ; gaz naturel ; et hydrogène.

17. Procédé selon l'une quelconque des revendications 1 à 16 **caractérisé en ce que** la fusion est réalisée dans un four à arc ouvert CC à une température située entre 1650 et 1750 °C.
